

## [54] PHOSPHONAMIDES

[76] Inventors: **Fred S. Eiseman, Jr.**, 516 Summit Ave., Maplewood; **Leslie M. Schenck**, 1558 Grouse Ln., Mountainside, both of N.J.; **John P. G. Beiswanger**, 720 Coleman St., Easton, Pa.

[22] Filed: Oct. 4, 1968

[21] Appl. No.: 765,001

[52] U.S. Cl. .... 260/945, 117/138.5, 260/974, 260/984

[51] Int. Cl. .... C07f 9/24

[58] Field of Search..... 260/945

## [56] References Cited

## UNITED STATES PATENTS

2,302,805 11/1942 Schüssler ..... 260/945 X

## OTHER PUBLICATIONS

Kondratev et al., Index Chemicus, Vol. 19, page 57137 (1965).

Primary Examiner—Lorraine A. Weinberger  
Assistant Examiner—Richard L. Raymond  
Attorney, Agent, or Firm—Walter C. Kehm; Samson B. Leavitt

## [57] ABSTRACT

Phosphonamide antistatic agents having the formula :



wherein R represents an alkyl phenyl, or alkyl-substituted phenyl radical having at least 7 carbon atoms, X represents hydrogen, methyl or ethyl, R<sub>1</sub> and R<sub>2</sub> are members of the group consisting of alkyl and hydroxy alkyl radicals of from 1-3 carbon atoms, R<sub>3</sub> is a hydroxy alkyl radical of from 1-4 carbon atoms, Y is an anion, m is an integer of from 1-10, n is an integer of from 1-2, and p is an integer of from 1-2, and the sum of n + p = 3.

7 Claims, No Drawings

1  
PHOSPHONAMIDES

The instant invention relates to new and useful compositions of matter which function as antistatic agents when coated on synthetic and natural fibers, e.g. polyester fibers, acetate rayons, wool, polyolefins, and the like, and to the method of use therefor. In particular, the instant invention is directed to substituted phosphonamides which exhibit antistatic properties, which phosphonamides are prepared by the condensation of alkyl and aryl polyethyleneoxy chlorophosphonates with a substituted alkyl diamine, followed by acidification and alkoxylation.

The commercial importance of the synthetic fiber industry has greatly emphasized the importance of antistatic agents and finishes since synthetic fibers, e.g., polyester fibers, acrylics, vinyls, etc. are notorious static electricity generators. While other fibers, e.g., cotton or viscose, do not generate the static electricity to any great extent under normal humidity conditions, and fibers such as acetate, rayon, and wool are only moderate generators, necessitating only some precautionary measures in the processing mill, e.g., a controlled high humidity, synthetic fibers such as mentioned above are not easily treated to control static electricity buildup.

While several non-durable finishes have been proposed which are moderately effective in eliminating static buildup on these synthetic fibers, few have been proposed which are completely satisfactory durable antistats. Most finishes employed to eliminate static buildup on synthetic fibers fall into the category of true surfactants although there is no really distinct similarity or correlation between surface activity and antistatic action.

In general, antistatic agents function in two ways, both of which improve the electrical conductivity of the fiber surface. Such antistatic agents are either reasonably good conductors of electricity themselves, or they are hygroscopic and help concentrate atmospheric moisture on the fibers.

The majority of antistatic agents fall into one of the following three categories: (1) polyhydroxy and polyethyleneoxy non-ionic compounds; (2) cationic, or neutral nitrogenous compounds with a hydrophobic moiety in their structure; (3) long-chain phosphates, phosphonates, or other oxygenated phosphorus derivatives. Additional types include sulfonated oils and ester emulsions, and other fiber lubricant emulsions which depend on the particular emulsifying agent used for their antistatic effect.

Long-chain quaternary ammonium salts have a marked antistatic action and are widely used in this capacity. These quaternaries, in common with numerous antistatic finishes, are frequently used in combination with auxiliary agents which may themselves be antistats, or serve the secondary purpose of binding the finish to the fiber, as disclosed in U.S. Pat. No. 2,463,282. The water-insoluble salts of higher amines, together with polystyrene sulfonates, are described in U.S. Pat. No. 2,700,001 as nylon antistats. The use of phosphorus compounds in antistatic capacities is given in U.S. Pat. Nos. 2,575,382; 2,575,399, and 2,676,122. Hygroscopic salts, such as cyclohexylamine lactate, are disclosed in Ger. Pat. No. 840,694, while the use of polyethoxylated fatty acids and alcohols as antistatic agents

for polypropylenes as well as fibers, is reported in U.S. Pat. No. 2,525,691.

In accordance with the instant invention, it has now been found that when one incorporates certain compounds which contain a phosphonamide structure within the molecule and, more specifically, those phosphonamide compounds derived from chlorophosphonate of an alkoxyated primary or secondary alcohol or alkyl phenol and gamma-dialkylaminopropylamine, show excellent antistatic properties when applied to synthetic fibers. These novel phosphonamides impart not only antistatic properties associated with both an amide linkage and that imparted by a quaternary configuration but, in addition, they also impart the desirable properties and characteristics of polyethoxylated hydrophobes. Unexpectedly, the combination of these chemical functions within a phosphonamide molecular structure provides an enhancement lacking when one simply admixes antistatic agents of the non-ionic and amide type.

It is, therefore, a principal object of the present invention to provide new and useful phosphonamide antistatic agents.

A further object of the present invention comprises the preparation of antistatic agents which have enhanced effectiveness with antistatic agents which contain an amide linkage and a polyalkoxylated hydrophobe.

Yet a further object of the instant invention is to prepare new and useful substituted phosphonamides which are derived from the chlorophosphonate of an alkoxyated primary or secondary alcohol or phenol and a substituted alkyl diamine.

Yet another object of the instant invention is to provide a process for the preparation of a new and useful antistatic agent, which process comprises the condensation of alkyl and aryl polyethyleneoxy chlorophosphonates with a substituted alkyl diamine, followed by acidification and alkoxylation.

Still further objects of the instant invention will become more apparent from the following detailed description thereof.

The new and useful antistatic agents of the instant invention correspond to the general formula:



wherein R represents an alkyl phenyl or alkyl-substituted-phenyl radical containing at least 7 carbon atoms, X represents hydrogen, methyl or ethyl, R<sub>1</sub> and R<sub>2</sub> represent alkyl or hydroxy alkyl radicals having from 1-3 carbon atoms, R<sub>3</sub> is a hydroxy alkyl radical having from 1-4 carbon atoms. Y is an anion, m is an integer of from 1-10, n is an integer of from 1-2 and p is an integer of from 1-2. In particular, R may be exemplified, but is not limited to, the following alkyl, phenyl or alkaryl radicals:

heptyl  
octyl  
nonyl  
decyl  
undecyl  
dodecyl  
tridecyl  
hexadecyl

octadecyl  
methylphenyl  
ethylphenyl  
butylphenyl  
hexylphenyl  
octylphenyl  
nonylphenyl  
decylphenyl  
dodecylphenyl  
pentadecylphenyl  
octadecylphenyl  
nonadecylphenyl  
phenyl

Exemplary alkyl and hydroxy alkyl radicals for  $R_1$  and  $R_2$  include:

methyl  
ethyl  
propyl  
isopropyl  
hydroxymethyl  
hydroxyethyl  
hydroxypropyl  
dihydroxypropyl, etc.

Exemplary hydroxy alkyl radicals for  $R_3$  include:

hydroxymethyl  
hydroxyethyl  
hydroxypropyl  
hydroxybutyl

dihydroxypropyl  
dihydroxybutyl, etc.

Exemplary anions for  $Z$  include:

halides  
chloride  
bromide  
iodide  
phosphates  
nitrates  
sulfates and the like.

In general, the novel phosphonamides of the instant invention are prepared by the condensation of alkyl and aryl polyethyleneoxy chlorophosphonates with a substituted alkyl diamine followed by acidification and alkoxylation. More specifically, in our preferred synthesis, a commercial straight chain aliphatic alcohol admixture comprising approximately 5%  $C_{11}$ , 25%  $C_{12}$ , 30%  $C_{13}$ , 30%  $C_{14}$  and 10%  $C_{15}$  is reacted with an alkylene oxide using an alkaline catalyst at 120°–150°C. and 1–30 psig until one to ten moles of the oxide is added. In place of the alkaline catalyst, acidic catalysts such as  $BF_3$ ,  $H_3PO_4$  and the like can be used. Secondary alcohols such as 2-decanol, 3-decanol, 4-decanol, 3-dodecanol, 4-tetradecanol, 6-hexadecanol, and the like or their admixtures as well as alkylphenols such as octylphenol, linear decyl phenol, branched dodecylphenol, etc, can be substituted for the primary aliphatic alcohol. The resultant alkyl or alkyl-aryl polyalkyleneoxyalkanol is then reacted with phosphorous oxychloride to form the corresponding mono or di alkyl or alkylaryl polyalkyleneoxy chlorophosphonate and the latter compound converted to its phosphonamide by reaction with gamma dialkylaminopropylamine. This latter derivative is acidified and reacted with an alkylene oxide to form its quaternary ammonium salt.

The above process is in general in accordance with the following reactions:



In general a substantially equivalent amount of reactants is employed and the reaction is carried out by agitating the ethoxylate mixture while the phosphorous oxy chloride is added dropwise until the reaction is close to being theoretically completed.

The alkyl, phenyl or alkaryl polyalkyleneoxy chlorophosphonate is further reacted with a substantially equivalent amount of gamma dialkyl or dialkanol aminopropyl amine to produce a substituted amide in accordance with the following reaction:



The novel substituted amide produced by reaction III can then be quaternized by reaction with an alkylene oxide or hydroxy substituted alkylene oxide in the presence of an acid. Such reaction may be represented as follows:



In the above reactions  $R$ ,  $R_1$ ,  $R_2$ ,  $R_3$ ,  $X$ ,  $m$ ,  $n$ ,  $P$ , and  $Y$  are previously defined.  $A$  represents an integer of from 1 to 5.

The new and useful antistatic agents of the present invention have been found to have unexpectedly advantageous antistatic properties, particularly when applied to synthetic fibers, such as polyesters, acrylics, polyolefins, polyamides, etc. Such antistatic agents have been found to reduce and maintain the electrostatic charges for extended periods of time below a potential of 3 kilovolts.

The present invention will now be described by reference to the following specific examples. Such examples are presented for purposes of illustration only, and the present invention is in no way to be deemed as limited thereto.

#### EXAMPLE 1

a. To a round bottom flask was charged a total of 288 parts by weight of an ethoxylate (1.85 moles EO) of a  $C_{11}$ – $C_{15}$  straight chain primary alcohol admixture calculated as a 209 M.W. average and having the compo-

sition 5% C<sub>11</sub>, 25% C<sub>12</sub>, 30% C<sub>13</sub>, 30% C<sub>14</sub> and 10% C<sub>15</sub>. The ethoxylate was agitated at ambient temperature (20°-30°C.) while 77 parts phosphorous oxychloride (0.5 mol.) were dropped in over about 1.5 to 2.0 hours. After addition of phosphorous oxychloride was completed the batch was heated to 60°-70°C. and held 1 hour. Dry nitrogen was then bubbled through the mixture and the temperature was maintained for one hour. Samples were then run and repeated at one hour intervals until the percent chlorine on hydrolyzed sample showed as low as theoretical.

b. To a beaker equipped with agitator, two dropping funnels, thermometer and a pH meter were charged 500 ml. water and 91 gms. dimethyl propylene diamine (0.9 mole). These materials were agitated at room temperature while 591 gms. of the chlorophosphonate (0.9 mol) prepared in (a) and 30% NaOH were dropped in simultaneously over about 1 to 1.5 hours at such a rate as to maintain the pH between 10.5 to 11.0. A total of 130 gms. 30% NaOH was required. After all reactants were added the batch was agitated 15 minutes at room temperature and then brought to pH 9.0 with CP HCl.

A total of 12.0 gms were required. The product was then stripped of water at 40 mm. pressure and the residue was filtered. The yield was 557 gms. Theoretical yield was 0.9 × 722 = 650 gms. so the % yield was 85.8.

c. To a 2-liter 4 necked flask with joints clamped for slight pressure were charged 430 gms. (0.6 mol) of the above phosphonamide, 300 ml. H<sub>2</sub>O and 300 gms. isopropanol. Then 40 gms. 85% phosphoric acid were added to bring pH to 3.0 to 3.5. Materials were agitated at 50°-60°C. and purged with N<sub>2</sub>. Ethylene oxide (28 gms. from cylinder) were added. A total of 24.0 gms. were absorbed.

The product was stripped to 110°C. pot temperature under line vacuum and then filtered.

The weight of the final product was 437 gms.

% nitrogen = 3.0

Theory = 3.3

The product generally corresponds to the formula:



d. The quaternary formed above was applied from MeOH/CCl<sub>4</sub> (520 mls/1000 mls) solvent mixture to Nylon Faille and Dacron swatches at 1.25% application rate according to AATCC Standard Test Method 76-1959.

The swatches were conditioned at 72°F. and 50% relative humidity for at least 24 hours and the resistivity measured. Results were as follows:

Log Ohms/Square

|                            | Nylon Faille | Dacron |
|----------------------------|--------------|--------|
| Control (Untreated Fabric) | 14.02        | 13.46  |
| Quaternary phosphonamide   | 8.79         | 8.65   |

## EXAMPLE II

The product was prepared as in Parts (a) and (b) of Example I.

c. To a 2 liter 4 necked flask with joints clamped for slight pressure were charged 430 gms (0.6 mole) of the above phosphonamide, 300 ml H<sub>2</sub>O and 300 gms isopropanol. Then 108 gms 1/1 H<sub>2</sub>O/C.P. HNO<sub>3</sub> were added to bring pH to 3.0 to 3.5. Materials were agitated at 50°-60°C. and purged with N<sub>2</sub>. Ethylene oxide (29 gms from cylinder) were added. A total of 22.5 gms were absorbed.

The product was stripped to 110°C. pot temperature under line vacuum and then filtered.

The weight of the final product was 451 gms.

% Nitrogen = 4.8

Theory = 5.07

The product generally corresponds to the formula:



d. The quaternary formed above was applied from MeOH/CCl<sub>4</sub> (520 mls/1000 mls) solvent mixture to Dacron and to cotton swatches at 1.25% application rate according to AATCC Standard Test Method 76-1959.

The swatches were conditioned at 72°F. and 50% relative humidity for at least 24 hours and the resistivity measured. Results were as follows:

Log Ohms/Square

|                          | Dacron | Cotton |
|--------------------------|--------|--------|
| Control                  | 13.46  | 14.24  |
| Quaternary Phosphonamide | 8.96   | 8.87   |

## EXAMPLE III

The product was prepared as in Parts (a) and (b) of Example I.



c. To a joints 2 liter 4 necked flask with hoints clamped for slight pressure were charged 430 gms (0.6 mole) of the above carbamate, 300 ml H<sub>2</sub>O and 300 gms isopropanol. Then 47.5 gms H<sub>2</sub>SO<sub>4</sub> were added to bring pH to 3.0 to 3.5. Materials were agitated at 50°-60°C. and purged with N<sub>2</sub>. Ethylene oxide (30.0 gms from cylinder) were added. A total of 26 gms were absorbed.

The product was stripped to 110°C. put temperature under line vacuum and then filtered.

The weight of the final product was 440 gms.

% Nitrogen = 3.1

Theory = 3.3

the product generally corresponds to the formula:



d. The quaternary formed above was applied from

5 The product generally corresponds to the formula:



MeOH CCl<sub>4</sub> (520 mls 1,000 mls) solvent mixture to 10 Nylon Faile and Polypropylene swatches at 1.25% application rate according to AATCC Standard Test Method 76-1959.

The swatches were conditioned at 72°F and 50% relative humidity for at least 24 hours and the resistivity 15 measured. Results were as follows:

|                          | Log Ohms/Square |               |
|--------------------------|-----------------|---------------|
|                          | Nylon Faile     | Polypropylene |
| Control                  | 14.02           | 14.64         |
| Quaternary Phosphonamide | 8.85            | 9.10          |

20  
25

|                          | Log Ohms/Square |             |
|--------------------------|-----------------|-------------|
|                          | Dacron          | Nylon Faile |
| Control                  | 13.46           | 14.02       |
| Quaternary phosphonamide | 8.92            | 9.08        |

#### EXAMPLE IV

a. To a round bottom flask was charged a total of 306 parts by weight of an ethoxylate (4.0 mole E.O.) of octyl alcohol. The ethoxylate was agitated at ambient temperature (20°-30°C) while 77 parts phosphorous oxychloride (0.5 ml) were dropped in over about 1.5 to 2.0 hours. After addition of phosphorous oxychloride was completed the batch was heated to 60°-70°C and held one hour longer. Samples were then run and repeated at one hour intervals until the percent chlorine on hydrolyzed samples showed as low as theoretical.

b. To a breaker equipped with agitator, two dropping funnels, thermometer and a pH meter were charged 500 ml water and 91 gms dimethyl propylene diamine (0.9 mole). These materials were agitated at room temperature while 623 gms of the phosphonamide (0.9 mol) prepared in (a) and 30% NaOH were dropped in simultaneously over about 1 to 1.5 hours at such a rate as to maintain the pH between 10.0 to 10.5. A total of 108 gms 30% NaOH was required. After all reactants were added the batch was agitated 15 minutes at room temperature and then brought to pH 9.0 with CP HCl. A total of 13.0 gms were required. The product was then stripped of water at 40 mm pressure and the residue was filtered. The yield was 552 gms. Theoretical yield was  $0.9 \times 758 = 682$  gms so the % yield was 80.9.

c. To a 1 liter 4 necked flask with joints clamped for a slight pressure were charged 455 gms (0.6 mole) of the above phosphonamide 350 ml H<sub>2</sub>O and 45 gms H<sub>3</sub>PO<sub>4</sub> to bring pH to 3.0 to 3.5. Materials were agitated at 50°-60°C and purged with N<sub>2</sub>. Ethylene oxide (33gms from cylinder) were added. A total of 26 gms were absorbed.

The product was stripped to 110°C pot temperature under line vacuum and then filtered.

The weight of the final product was 460 gms.

10 d. The quaternary formed above was applied from MeOH CCl<sub>4</sub> (52.0 mls 1,000 mls) solvent mixture to Dacron and Nylon Faile swatches at 2.5% application rate according to AATCC Standard Test Method 76-1959.

The swatches were conditioned at 72°F and 50% relative humidity for at least 24 hours and the resistivity measured.

15 Results were as follows:

#### EXAMPLE V

a. To a round bottom flask was charged a total of 660 parts by weight of an ethoxylate (10.0 moles EO) of nonyl phenol. The ethoxylate was agitated at ambient temperature (20°-30°C) while 77 parts phosphorous oxychloride (0.5 mol.) were dropped in over about 1.5 to 2.0 hours. After addition of phosphorous oxychloride was completed the batch was heated to 60°-70°C and held 1 hour. Dry nitrogen was then bubbled through the mixture and the temperature was maintained for one hour. Samples were then run and repeated at one hour intervals until the percent chlorine on hydrolyzed sample showed as low as theoretical.

b. To a beaker equipped with agitator, two dropping funnels, thermometer and a pH meter were charged 700 ml water and 91 gms dimethyl propylene diamine (0.9 mole). These materials were agitated at room temperature while 1,260 gms of the chlorophosphonate (0.9 mol.) prepared in (a) and 30% NaOH were dropped in simultaneously over about 1 to 1.5 hours at such a rate as to maintain the pH between 10.5 to 11.0. A total of 150 gms 30% NaOH was required. After all reactants were added the batch was agitated 15 minutes at room temperature and then brought to pH 9.0 with CP HCl. A total of 12.0 gms were required. The product was then stripped of water at 40 mm pressure and the residue was filtered. The yield was 1,053 gms. Theoretical yield was  $0.9 \times 1466 = 1,320$  gms so the % yield was 79.8.

c. To a 2 liter 4 necked flask with joints clamped for slight pressure were charged 880 gms (0.6 mol) of the above phosphonamide, 400 ml H<sub>2</sub>O and 400 gms Isopropanol. Then 40 gms 85% Phosphoric Acid were added to bring pH to 3.0 to 3.5. Materials were agitated at 50°-60°C and purged with N<sub>2</sub>. Ethylene oxide (28 gms. from cylinder) were added. A total of 24.0 gms were absorbed.

60 The product was stripped to 110°C pot temperature under line vacuum and then filtered.

The weight of the final product was 886 gms.

% Nitrogen = 1.55

Theory = 1.74

The product generally corresponds to the formula:



d. The quaternary formed above was applied from MeOH:CCl<sub>4</sub> (520 mls 1000 mls) solvent mixture to Polypropylene and Dacron swatches at 1.25% application rate according to AATCC Standard Test Method 15 76-1959.

The swatches were conditioned at 72°F and 50% relative humidity for at least 24 hours and the resistivity

measured. Results were as follows:

|                          | Log Ohms/Square |        |
|--------------------------|-----------------|--------|
|                          | Polypropylene   | Dacron |
| Control                  | 14.64           | 13.46  |
| Quaternary phosphonamide | 8.98            | 8.74   |

#### EXAMPLE VI

a. To a round bottom flask was charged a total of 288 parts by weight of an ethoxylate (1.85 moles EO) of a C<sub>11</sub>-C<sub>15</sub> straight chain primary alcohol admixture calculated as a 209 M.W. average and having the composition 5% C<sub>11</sub>, 25% C<sub>12</sub>, 30% C<sub>13</sub>, 30% C<sub>14</sub> and 10% C<sub>15</sub>. The ethoxylate was agitated at ambient temperature (20°-30°C) while 153 parts phosphorus oxychloride (1.0 mol.) were dropped in over about 1.5 to 2.0 hours. After addition of phosphorous oxychloride was completed the batch was heated to 60°-70°C and held 1 hour. Dry nitrogen was then bubbled through to mixture and the temperature was maintained for 1 hour. Samples were then run and repeated at 1 hour intervals until the percent chlorine on hydrolyzed sample 45 showed as low as theoretical.

b. to a breaker equipped with agitator, two dropping funnels, thermometer and a pH meter were charged 500 ml water and 182 gms dimethyl propylene diamine (1.8 mole). These materials were agitated at room temperature while 364 gms of the chlorophosphonate (0.9 mol) prepared in (a) and 30% NaOH were dropped in simultaneously over about 1 to 1.5 hours at such a rate as to maintain the pH between 10.5 to 11.0. A total of 230 gms 30% NaOH was required. After all reactants were added the batch was agitated 15 minutes at room temperature and then brought to pH 9.0 with CP HCl. A total of 22.0 gms were required. The product was then stripped of water at 40 mm pressure and the residue was filtered. The yield was 402 gms. Theoretical yield was 0.9 × 536 = 482 gms so the % yield was 83.3.

c. To a 1 liter 4 necked flask with joints clamped for slight pressure were charged 322 gms (0.6 mol) of the above phosphonamide, 200 ml H<sub>2</sub>O and 200 gms iso-

propanol. Then 45 gms 85% Phosphoric Acid were added to bring pH to 3.0 to 3.5. Materials were agitated at 50°-60°C and purged with N<sub>2</sub>. Ethylene oxide (54 gms. from cylinder) were added. A total of 47.0 gms were absorbed.

The product was stripped to 110°C pot temperature under line vacuum and then filtered.

The weight of the final product was 470 gms.

% Nitrogen = 6.71 Theory = 6.85

The product generally corresponds to the formula:



d. The quaternary formed above was applied from MeOH:CCl<sub>4</sub> (520 mls 1000 mls) solvent mixture to cotton and Dacron swatches at 1.25% application rate according to AATCC Standard Test Method 76-1959.

The swatches were conditioned at 72°F and 50% relative humidity for at least 24 hours and the resistivity measured. Results were as follows:

|                          | Log Ohms/Square |        |
|--------------------------|-----------------|--------|
|                          | Cotton          | Dacron |
| Control                  | 14.24           | 13.46  |
| Quaternary phosphonamide | 8.68            | 8.73   |

What is claimed is:

1. A compound of the formula:



wherein R represents an alkyl, phenyl or alkylsubstituted phenyl radical having 7 to about 25 carbon atoms, X represents hydrogen, methyl or ethyl, R<sub>1</sub> and R<sub>2</sub> are members of the group consisting of alkyl and hydroxy alkyl radicals of from 1-3 carbon atoms, R<sub>3</sub> is a hydroxy alkyl radical of from 1-4 carbon atoms, Y is an anion, m is an integer of from 1-10, n is an integer of from 1-2, and p is an integer of from 1-2, and the sum of n + p = 3.

2. A compound of the formula:



3. A compound of the formula:



6. A compound of the formula:



4. A compound of the formula:



7. A compound of the formula:



5. A compound of the formula:



\* \* \* \* \*

UNITED STATES PATENT OFFICE  
CERTIFICATE OF CORRECTION

PATENT NO. : 3,856,895

DATED : December 24, 1974

INVENTOR(S) : Fred S. Eisman, Jr.; L. M. Schenck; John P. G. Beiswanger

It is certified that error appears in the above-identified patent and that said Letters Patent are hereby corrected as shown below:

On the front page, after the listing of inventors, insert

--Assignee: GAF Corporation  
New York, N.Y.--

Signed and Sealed this  
*twenty-fourth Day of February 1976*

[SEAL]

*Attest:*

**RUTH C. MASON**  
*Attesting Officer*

**C. MARSHALL DANN**  
*Commissioner of Patents and Trademarks*